

[54] PROCESS FOR THE RESIN FINISHING OF CELLULOSIC FABRICS AND CELLULOSIC BLEND FABRICS WITH SIMULTANEOUS IMPROVEMENT OF THEIR AFFINITY FOR OPTICAL BRIGHTENERS

[75] Inventors: **Kurt Poppenwimmer**, Allschwil/Basel-Land; **Hilmar Roedel**, Therwil/Basel-Land, both of Switzerland

[73] Assignee: **Sandoz Ltd.**, Basle, Switzerland

[22] Filed: June 30, 1971

[21] Appl. No.: 158,518

[30] Foreign Application Priority Data

July 10, 1970 Switzerland..... 10452/70

[52] U.S. Cl..... 117/33.5 T, 8/115.6, 8/116.2, 117/139.4, 117/139.5 A, 117/139.5 CQ

[51] Int. Cl..... C09j 3/00, D06m 13/34

[58] Field of Search .. 117/33.5 T, 139.4, 139.5 CQ, 117/139.5 A; 260/29.6 HN, 29.6 B, 29.6 WA, 29.6 RB; 8/116.2, 1 W, 100, 115.5,

115.6, 116.3; 252/301.2 W

[56]

References Cited

UNITED STATES PATENTS

|           |         |                      |               |
|-----------|---------|----------------------|---------------|
| 3,232,691 | 2/1966  | Wilhelm et al.....   | 117/33.5 T X  |
| 3,238,166 | 3/1966  | Kawai et al.....     | 117/139.4 X   |
| 3,322,569 | 5/1967  | Faulhaber et al..... | 117/139.4     |
| 3,402,987 | 9/1968  | Dalton et al.....    | 260/29.6 HN X |
| 3,533,728 | 10/1970 | Shippee et al.....   | 8/17 X        |

Primary Examiner—Alfred L. Leavitt

Assistant Examiner—Caleb Weston

Attorney, Agent, or Firm—Gerald D. Sharkin

[57]

ABSTRACT

A process for the resin finishing of cellulosic blend fabrics with improvement of their affinity for anionic optical brighteners by treating the fabrics with a solution of a) an N-methylol or N-alkoxymethyl compound b) an acid curing catalyst c) a copolymer consisting of vinyl pyrrolidone units and at least 5.5 weight percent vinyl alcohol units and curing by dry heat treatment at 120°-180°C.

11 Claims, No Drawings

PROCESS FOR THE RESIN FINISHING OF  
CELLULOSIC FABRICS AND CELLULOSIC BLEND  
FABRICS WITH SIMULTANEOUS IMPROVEMENT  
OF THEIR AFFINITY FOR OPTICAL  
BRIGHTENERS

5

White fabrics of cellulosic fibre and blend fabrics of a cellulosic and another fibre which have been finished with resins take on a greyish appearance after a much shorter period of use than in the case with fabrics without a resin finish. The main reason is that the optical brightener subsequently applied to the fabric is not fixed to be fully resistant to washing. Unlike fabrics without a resin finish, resin finished fabrics absorb very little or no optical brighteners from the wash baths, and after they have been in use for some length of time and repeatedly washed they lose their original whiteness. This greying of the fabric is promoted by the reabsorption from the wash bath of detached soil particles.

To prevent greying, resin finished cellulosic and cellulosic blend fabrics are often finished additionally with soil release agents, one function of which is to check the re-absorption of soil particles from the wash liquor. However, soil release agents have no or only very low affinity for the optical brighteners in the detergents used for domestic washing.

It has now been found that white cellulosic and cellulosic blend fabrics can be resin finished and their affinity for anionic optical brighteners increased at the same time by padding the fabric with an aqueous solution of

- a. an N-methylol or N-alkoxymethyl compound,
- b. an acid catalyst as curing agent for the N-methylol or N-alkoxymethyl compound and
- c. a copolymer consisting of vinyl pyrrolidone units and

at least 5.5 weight percent vinyl alcohol units, followed if desired by drying and then by curing by dry heat treatment at 120°-180°C.

The invention relates further to aqueous solutions of

- a. an N-methylol or N-alkoxymethyl compound,
- b. an acid curing agent for the N-methylol or N-alkoxymethyl compound and
- c. a copolymer consisting of vinyl pyrrolidone units and at least 5.5 weight percent vinyl alcohol units.

The suitable anionic optical brighteners include those of the stilbene triazinyl series, in particular those of formula



where

Me stands for a monovalent cation ( $\text{Na}^+$ ,  $\text{K}^+$ ,  $\text{NH}_4^+$ ,  $\text{NH}_2^+-\text{C}_2\text{H}_5\text{OH}$  etc.),

$X_1$  and  $X_2$ , independently of each other, for alkoxy, alkylamino, hydroxyalkylamino, N-alkyl-N-hydroxy-alkylamino, aminocarbonylalkylamino, N-alkyl-N-hydroxyalkylamino, N,N-di(hydroalkyl)amino, N-hydroxyalkyl-N-cyanoalkyl, N-

|   | $X_1$                                       | $X_2$                                       | $Y_1$                                | $Y_2$ | Me               |
|---|---------------------------------------------|---------------------------------------------|--------------------------------------|-------|------------------|
| A | —NH— $\text{C}_2\text{H}_5\text{OH}$        | —NH— $\text{C}_2\text{H}_5\text{OH}$        |                                      |       | Na               |
| B | —NH— $\text{C}_2\text{H}_5\text{OH}$        | —NH— $\text{C}_2\text{H}_5\text{OH}$        | Same as above                        |       | $\text{NH}_2^+$  |
| C | —NH— $\text{C}_2\text{H}_5\text{OH}$        | —NH— $\text{C}_2\text{H}_5\text{OH}$        | —NH— $\text{C}_2\text{H}_5\text{OH}$ |       | Na               |
| D | —NH— $\text{C}_2\text{H}_5\text{OH}$        | —NH— $\text{C}_2\text{H}_5\text{OH}$        | —NH— $\text{C}_2\text{H}_5\text{OH}$ |       | K                |
| E | —NH— $\text{C}_2\text{H}_5\text{OH}$        | —NH— $\text{C}_2\text{H}_5\text{OH}$        | —NH— $\text{C}_2\text{H}_5\text{OH}$ |       | Na               |
| F | —NH— $\text{C}_2\text{H}_5\text{OH}$        | —NH— $\text{C}_2\text{H}_5\text{OH}$        |                                      |       | Na               |
| G | —NH— $\text{C}_2\text{H}_5\text{OH}$        | —NH— $\text{C}_2\text{H}_5\text{OH}$        |                                      |       | Na               |
| H | —NH— $\text{C}_2\text{H}_5\text{OH}$        | —NH— $\text{C}_2\text{H}_5\text{OH}$        |                                      |       | Na               |
| I | —NH— $\text{CH}_2\text{—CHOH—CH}_2\text{—}$ | —NH— $\text{CH}_2\text{—CHOH—CH}_2\text{—}$ |                                      |       | Na               |
|   | —NH— $\text{CH}_2\text{—CHOH—CH}_2\text{—}$ | —NH— $\text{CH}_2\text{—CHOH—CH}_2\text{—}$ |                                      |       | OCH <sub>3</sub> |

Table - Continued

|   | X <sub>1</sub>                                           | X <sub>2</sub>                                           | Y <sub>1</sub>                                           | Y <sub>2</sub>           | Me |
|---|----------------------------------------------------------|----------------------------------------------------------|----------------------------------------------------------|--------------------------|----|
| K | —NH—CH <sub>2</sub> —CH(OH)—CH—                          | —NH—CH <sub>2</sub> —CHOH—CH <sub>3</sub>                | —NH—CH <sub>2</sub> —CH(OH)—CH <sub>3</sub>              | —NH—CH <sub>2</sub> —NH— | Na |
| L | —NH—CH <sub>2</sub> —CH(OH)—CH <sub>3</sub>              | —NH—CH <sub>2</sub> —CHOH—CH <sub>3</sub>                | —NH—CH <sub>2</sub> —CH(OH)—CH <sub>3</sub>              | —NH—CH <sub>2</sub> —NH— | Na |
| M | —NH—CH <sub>2</sub> —CH(OH)—CH <sub>3</sub>              | —NH—CH <sub>2</sub> —CHOH—CH <sub>3</sub>                | —NH—CH <sub>2</sub> —CH(OH)—CH <sub>3</sub>              | —NH—CH <sub>2</sub> —NH— | Na |
| N | —NH—CH <sub>2</sub> —CH(OH)—CH <sub>3</sub>              | —NH—CH <sub>2</sub> —CH(OH)—CH <sub>3</sub>              | —NH—CH <sub>2</sub> —CH(OH)—CH <sub>3</sub>              | —NH <sub>2</sub>         | Na |
| O | —NH—CH <sub>2</sub> —CH(OH)—CH <sub>3</sub>              | —NH—CH <sub>2</sub> —CH(OH)—CH <sub>3</sub>              | —NH—CH <sub>2</sub> —CH(OH)—CH <sub>3</sub>              | SO <sub>3</sub> Na       | Na |
| P | —N(C <sub>2</sub> H <sub>5</sub> OH) <sub>2</sub>        | —N(C <sub>2</sub> H <sub>5</sub> OH) <sub>2</sub>        | —N(C <sub>2</sub> H <sub>5</sub> OH) <sub>2</sub>        | —NH <sub>2</sub>         | Na |
| Q | —N(C <sub>2</sub> H <sub>5</sub> OH) <sub>2</sub>        | —N(C <sub>2</sub> H <sub>5</sub> OH) <sub>2</sub>        | —N(C <sub>2</sub> H <sub>5</sub> OH) <sub>2</sub>        | SO <sub>3</sub> Na       | Na |
| R | —N(C <sub>2</sub> H <sub>5</sub> OH) <sub>2</sub>        | —N(C <sub>2</sub> H <sub>5</sub> OH) <sub>2</sub>        | —N(C <sub>2</sub> H <sub>5</sub> OH) <sub>2</sub>        | —NH <sub>2</sub>         | Na |
| S | —N(C <sub>2</sub> H <sub>5</sub> OH) <sub>2</sub>        | —N(C <sub>2</sub> H <sub>5</sub> OH) <sub>2</sub>        | —N(C <sub>2</sub> H <sub>5</sub> OH) <sub>2</sub>        | SO <sub>3</sub> Na       | Na |
| T | —NH—CH <sub>2</sub> —CH <sub>2</sub> —CO—NH <sub>2</sub> | —NH—CH <sub>2</sub> —CH <sub>2</sub> —CO—NH <sub>2</sub> | —NH—CH <sub>2</sub> —CH <sub>2</sub> —CO—NH <sub>2</sub> | —NH—CH <sub>2</sub> —NH— | Na |
| U | —NH—CH <sub>2</sub> —CH <sub>2</sub> —CO—NH <sub>2</sub> | —NH—CH <sub>2</sub> —CH <sub>2</sub> —CO—NH <sub>2</sub> | —NH—CH <sub>2</sub> —CH <sub>2</sub> —CO—NH <sub>2</sub> | —NH <sub>2</sub>         | Na |
| V | —NH—C <sub>2</sub> H <sub>5</sub> OH                     | —NH—C <sub>2</sub> H <sub>5</sub> OH                     | —NH—C <sub>2</sub> H <sub>5</sub> OH                     | —NH <sub>2</sub>         | Na |
| W | —CH <sub>3</sub> O—                                      | —CH <sub>3</sub> O—                                      | —CH <sub>3</sub> O—                                      | —NH—CH <sub>2</sub> —NH— | Na |
| X | —CH <sub>3</sub> O—                                      | —CH <sub>3</sub> O—                                      | —CH <sub>3</sub> O—                                      | —NH—CH <sub>2</sub> —O—  | Na |
| Y | —CH <sub>3</sub> O—                                      | —CH <sub>3</sub> O—                                      | —CH <sub>3</sub> O—                                      | —NH—CH <sub>2</sub> —NH— | Na |

Table—Continued

|     | X <sub>1</sub>                                                           | X <sub>2</sub>                                                           | Y <sub>1</sub>                                                                     | Y <sub>2</sub>                                                                     | Me |
|-----|--------------------------------------------------------------------------|--------------------------------------------------------------------------|------------------------------------------------------------------------------------|------------------------------------------------------------------------------------|----|
| Z   | CH <sub>3</sub> NH—                                                      | CH <sub>3</sub> NH—                                                      |                                                                                    |                                                                                    | Na |
| AA  | —N(C <sub>2</sub> H <sub>5</sub> OH) <sub>2</sub>                        | —N(C <sub>2</sub> H <sub>5</sub> OH) <sub>2</sub>                        |                                                                                    |                                                                                    | Na |
| AB  | CH <sub>3</sub><br>—N—<br>C <sub>2</sub> H <sub>5</sub> OH               | CH <sub>3</sub><br>—N—<br>C <sub>2</sub> H <sub>5</sub> OH               | NaO <sub>3</sub> S—<br>S O <sub>3</sub> Na<br>—NH—C <sub>2</sub> H <sub>5</sub> OH | NaO <sub>3</sub> S—<br>S O <sub>3</sub> Na<br>—NH—C <sub>2</sub> H <sub>5</sub> OH | Na |
| AC  | CH <sub>3</sub> O—                                                       | CH <sub>3</sub> O—                                                       | —NH—C <sub>2</sub> H <sub>5</sub> OH                                               | —NH—C <sub>2</sub> H <sub>5</sub> OH                                               | Na |
| AD  | —N(C <sub>2</sub> H <sub>5</sub> OH) <sub>2</sub>                        | —N(C <sub>2</sub> H <sub>5</sub> OH) <sub>2</sub>                        | NaO <sub>3</sub> S—<br>S O <sub>3</sub> Na                                         | NaO <sub>3</sub> S—<br>S O <sub>3</sub> Na                                         | Na |
| AE  | CH <sub>3</sub><br>—N—<br>C <sub>2</sub> H <sub>5</sub> OH               | CH <sub>3</sub><br>—N—<br>C <sub>2</sub> H <sub>5</sub> OH               | NaS <sub>3</sub> S—<br>—NH—<br>C <sub>2</sub> H <sub>5</sub> OH                    | NaO <sub>3</sub> S—<br>—NH—<br>C <sub>2</sub> H <sub>5</sub> OH                    | Na |
| AF  | C <sub>2</sub> H <sub>5</sub> O—                                         | C <sub>2</sub> H <sub>5</sub> O—                                         | —NH—C <sub>2</sub> H <sub>5</sub> OH                                               | —NH—C <sub>2</sub> H <sub>5</sub> OH                                               | Na |
| AG  | C <sub>2</sub> H <sub>5</sub><br>—N—<br>C <sub>2</sub> H <sub>5</sub> OH | C <sub>2</sub> H <sub>5</sub><br>—N—<br>C <sub>2</sub> H <sub>5</sub> OH | —NH <sub>2</sub>                                                                   | —NH <sub>2</sub>                                                                   | Na |
| AII | Same as above                                                            | —NH—<br>C <sub>2</sub> H <sub>5</sub> OH                                 | —NH <sub>2</sub>                                                                   | —NH <sub>2</sub>                                                                   | Na |
| AI  | CH <sub>3</sub> O—                                                       | CH <sub>3</sub> O—                                                       | NaO <sub>3</sub> S—<br>—NH—<br>C <sub>2</sub> H <sub>5</sub> OH                    | NaO <sub>3</sub> S—<br>—NH—<br>C <sub>2</sub> H <sub>5</sub> OH                    | Na |
| AK  | CH <sub>3</sub> NH—                                                      | C <sub>2</sub> H <sub>5</sub> NH—                                        | Same as above                                                                      | —NH <sub>2</sub>                                                                   | Na |
| AL  | C <sub>2</sub> H <sub>5</sub> —CO—NH <sub>2</sub>                        | C <sub>2</sub> H <sub>5</sub> —CO—NH <sub>2</sub>                        | —NH—<br>C <sub>2</sub> H <sub>5</sub> —CO—NH <sub>2</sub>                          | —NH—<br>C <sub>2</sub> H <sub>5</sub> —CO—NH <sub>2</sub>                          | Na |
| AM  | Same as above                                                            | Same as above                                                            | CH <sub>3</sub><br>—NH—<br>C <sub>6</sub> H <sub>5</sub>                           | CH <sub>3</sub><br>—NH—<br>C <sub>6</sub> H <sub>5</sub>                           | Na |

hydroxyalkyl-N-aminocarbonylalkyl, morpholine or piperidine radicals, and  $Y_1$  and  $Y_2$ , independently of each other, for aryloxy radicals of the benzene series, amino, alkylamino or arylamino groups of the benzene, naphthalene, or diphenyl series, in which alkyl and alkoxy may contain one to six carbon atoms and the aryl radicals may bear substituents such as alkyl, alkoxy, acylamino, sulphonic acid or carboxylic acid groups or halogen atoms. The products listed in Table I are representative members of this group of optical brighteners.

The following are examples of further suitable optical brighteners:

sodium 3,7-diacylaminodibenzothiophene dioxide-2,8-disulphonate, such as



where  $R_1$  in both positions represents



derivatives of 7-aminocomarin such as



derivatives of stilbenyl naphthotriazole such as



|    |           |           |           |       |
|----|-----------|-----------|-----------|-------|
| AR | $R_2$     | $R_3$     | $R_4$     | $R_5$ |
| AS | $-SO_3Na$ | $H$       | $-SO_3Na$ | $H$   |
| AT | $H$       | $-SO_3Na$ | $H$       | $H$   |
| AU | II        | $-SO_3Na$ | $H$       | $H$   |

derivatives of dehydrothiotoluidine such as



derivatives of oxacyanine such as 3, 3', 5, 5', 7, 7'-hexamethoxyacyanine-p-sulphonate = AW  
 derivatives of bis-azoles such as the sodium salt of sulphonated 2,2'-bis-[(phenyl vinylidene)-6,6'-oxazole] = AX  
 derivatives of sulphonated 2,2'-bis-[(phenyl vinylide-

ne)-6,6'-thiazole] = AY  
 derivatives of sulphonated 2,2'-bis-[(phenyl vinylidene)-6,6'-imidazole] = AZ

derivatives of diphenylazoles such as the sodium salt of sulphonated-2-styryl-5-phenyloxazole = BA  
 derivatives of sulphonated 2-naphthyl-5-phenylthiazole = BB  
 derivatives of sulphonated 2-naphthyl-5-phenylimidazole = BC

10 derivatives of an  $\alpha$ ,  $\beta$ -di-(benzimidazyl)-ethylene such as the sodium salt of sulphonated  $\alpha$ , $\beta$ -di-(benzimidazyl-2)-ethylene = BD  
 derivatives of diphenylimidazolone such as the sodium salt of sulphonated 4,5-diphenylimidazole = BE.

15 The cellulosic fabrics for finishing by the present process may be of natural or regenerated cellulosic fibre (cotton, linen, hemp, ramie, jute or viscose rayon, cuprammonium rayon, polynotic fibre), or blends of a cellulosic fibre and a natural fibre such as wool or silk or a synthetic fibre such as polyamide, polyurethane, polyacrylonitrile, polypropylene or preferably polyester fibre (polyethyleneterephthalate and the condensation product deriving from terephthalic acid and 1,4-dimethylol-cyclohexane).

20 Examples of suitable N-methylol and N-alkoxymethylol compounds are the polymethylol and polyalkoxymethyl compounds of triazinones, melamine, melamine derivatives, carbamates, urea and cyclic ureas of formula

30



35 where  $R_6$  represents



40



45



The polyalkoxymethyl compounds are produced by 50 etherification of polymethylol compounds using low molecular weight alcohols ( $CH_3OH$ ,  $C_2H_5OH$ ,  $n-C_4H_9OH$ ).

The curing agents suitable for the N-methylol compounds include the colourless salts formed by multivalent metals and strong inorganic acids, such as magnesium, zinc, cadmium and aluminium chlorides, bromides, nitrates, sulphates and other halides, zirconyl chloride, acid phosphates such as  $Mg(H_2PO_4)_2$ ,  $Al(H_2PO_4)_3$  and  $Zn(H_2PO_4)_2$ , the colourless salts of multivalent metals and organic acids, such as magnesium and zinc acetate and propionate; compounds which act acid

55 under the curing conditions, e.g. ammonium and amine salts such as ammonium bromide, chloride and sulphate, monoammonium and diammonium phosphate, ammonium oxalate, monomethyl, dimethyl and trimethyl aminohydrochloride, monoethyl, diethyl and triethyl aminohydrochloride, monoethanol, diethanol and triethanol aminohydrochloride, mono-, di- and tri-

propanol aminohydrochloride.

The N-methylol and N-alkoxymethyl compounds impart the actual finish, while the copolymers (c) improve the affinity for optical brighteners.

The degree of polymerization of the copolymers (c) is not critical so long as they are soluble in water at room temperature. Products polymerized to a high degree, with an average molecular weight greater than 50,000, or others of a low degree of polymerization with average molecular weights of 5,000 or less can be employed. But since high polymers form very viscous aqueous solutions and the low polymers are difficult to synthesize in a homogeneous state, preference is given to polymers and copolymers with molecular weights in the range of 5,000 to 50,000, e.g. 10,000 to 30,000.

Copolymers consisting of 5.5 to 55 weight percent of vinyl alcohol units and 94.5 to 45 weight percent vinylpyrrolidone units greatly increase the affinity.

The N-methylol and N-alkoxymethyl compounds are best employed in the padding liquor in amounts of 50-150 g/l, or preferably 70-120 g/l. The curing agent is added in amounts of 5-30 g/l, preferably 10-20 g/l, in crystalline form. The amount of copolymer (c) is preferably 3-50 g/l, the optimum range being 7.5-30 g/l.

The curing temperature may range from 120°C to 180°C, but it is preferable to cure in the range of 140° to 160°C in order to accomplish curing speedily and obtain a high-quality finish.

After curing the fabric is washed off at 50° to 100°C to remove the unfixed portion of the products. The washing-off bath can be set with non-ionic or anionic detergents, along with alkalis such as sodium or potassium carbonate, sodium or potassium silicates, trisodium phosphate, tetrasodium or tetrapotassium pyrophosphate, or condensed phosphates. It may also contain per salts such as sodium perborate as bleaching agents.

The non-ionic detergents suitable for this purpose include the adducts of ethylene oxide or propylene oxide on hydrophobic compounds such as fatty alcohols, fatty acids, fatty acid amides, monoalkyl- and polyalkyl-phenols, monoalkyl- and polyalkynaphthols, alkylmercaptans, alkylthiophenols, saccharic acid esters, methylalkyl sulphoxides, N-oxides of alkyl-di (lower alkyl)-amines or phosphines, and the weakly basic adducts of ethylene oxide on fatty amines. Suitable anionic detergents include alkylbenzene sulphonates, alkyl sulphonates, primary and secondary alkyl sulphates, alkyl, alkylphenyl, dialkylphenyl, alkynaphthyl and dialkyl-naphthyl polyglycolether sulphates, phosphates and oxyacetates, fatty acid amides of 2-aminoethane sulphonate, 2-N-methylaminoethane sulphonate, 2-aminoethyl sulphate, aminobenzene sulphonates and aminoalkoxybenzene sulphonates.

Cellulosic fabrics and blend fabrics finished as described above have higher dry and wet crease resistance values than comparable unfinished fabrics, and show higher affinity for anionic optical brighteners such as those in domestic detergents which build up on the fabric from the wash bath.

A typical formulation for such a detergent is as follows:

20 percent active washing substance (see above)

2 percent lauroyl diethanolamide

40 percent condensed phosphate, e.g. sodium tripolyphosphate

- 5 percent sodium metasilicate  
5 percent sodium carbonate  
10 percent sodium sulphate  
2 percent carboxymethyl cellulose  
5 10 percent sodium perborate ( $\text{NaBO}_2 \cdot \text{H}_2\text{O}_2 \cdot 3\text{H}_2\text{O}$ )  
0.5 percent anionic optical brightener  
5.5 percent moisture etc.

A merit of the process described herein is that it lessens the loss of tensile strength caused by the resin finishing of the fabric.

In the following Examples, which illustrate the invention without limiting its scope, the parts and percentages are by weight and the temperatures in degrees centigrade.

15

#### EXAMPLE 1

A 50/50 percent blend fabric of cotton and polyester fibre is added with an aqueous solution containing per litre,

- 20 100 g dimethylolethylene urea (100 percent strength),  
30 g magnesium chloride  $\text{MgCl}_2 \cdot 6\text{H}_2\text{O}$  and  
15 g of a vinyl pyrrolidone-vinyl alcohol copolymer produced as described below.

- 25 The fabric is dried at 100° to 120° and the resin cured by treatment for 4 to 5 minutes at 160°C.

The fabric is washed 5 times at 98° with an aqueous solution of 5 g/l of a commercial detergent. The detergent has the composition given above, the active wash substance being sodium dodecylbenzenesulphonate, the condensed phosphate sodium tripolyphosphate and the anionic optical brightener the compound designated P in the above enumeration.

In comparison with a fabric finished without the copolymer, the fabric finished according to this process has a far higher degree of whiteness after five washes under the same conditions, as these values show:

#### Fluorimeter values

|                                                       |    |
|-------------------------------------------------------|----|
| Fabric finished by the present process                | 42 |
| Fabric finished without a copolymer                   | 11 |
| Similar results are obtained with 100% cotton fabric. |    |

- 40
- 45 The vinyl pyrrolidone-vinyl alcohol copolymer used here was produced as follows. 50 parts of vinyl acetate, 50 parts of vinyl pyrrolidone, 75 parts of demineralized water, 41 parts of methanol and 0.2 parts of  $\alpha, \alpha'$ -azoo-iso-butyric acid dinitrile are mixed in a nitrogen atmosphere. The mixture is raised to 60° in 30 to 40 minutes. The polymerization reaction is slightly exothermic and its progress can be recognized from the increase in viscosity. The mixture is stirred for 3 hours at 60° to 65° then a further 76 parts of demineralized water, 60 parts 50 of methanol and 0.08 parts of  $\alpha, \alpha'$ -azoo-iso butyric acid dinitrile are added and stirring continued for 5 hours at 60° to 65° till polymerization is complete. After the addition of 470 parts of methanol, 100 parts of a solution of 10 parts of 87 percent potassium hydroxide in 90 55 parts of methanol are dropped in slowly.

The temperature is slowly increased to 95° to 98° and in 6 hours a mixture of methanol, methyl acetate and water is distilled. The distilled methanol is replaced by water.

- 60 65 The product is 90 parts of colourless vinyl pyrrolidone-vinyl alcohol copolymer in solution in 510 parts of water. It consists of 34 percent vinyl alcohol units and 66 percent vinyl pyrrolidone units and in the fol-

lowing is termed copolymer 34/66.

The following polymers and copolymers can be synthesized in an analogous manner to the above:

| Designation | Composition                                 | Produced from                                   |
|-------------|---------------------------------------------|-------------------------------------------------|
| 82/18       | 82% vinyl alcohol,<br>18% vinyl pyrrolidone | 90% vinyl acetate,<br>10% 67% vinyl pyrrolidone |
| 67/33       | 67% vinyl alcohol,<br>33% vinyl pyrrolidone | 80% vinyl acetate,<br>20% vinyl pyrrolidone     |
| 18/82       | 18% vinyl alcohol,<br>82% vinyl pyrrolidone | 30% vinyl acetate,<br>70% vinyl pyrrolidone     |

### EXAMPLE 2

A cotton fabric is padded with a solution containing 75 g/l of a 1:1 mixture of dimethylolethylene urea and dimethylolpropylene urea, 20 g/l  $MgCl_2 \cdot 6H_2O$  and 7.5 g/l of one of the copolymers listed in Example 1. After intermediate drying at 100° to 120° the finish is cured by treatment for 5 minutes at 160°. The fabric is

washed, either once at 60° or 5 times at 98°, with the detergent used in Example 1 at a concentration of 5 g/l, then rinsed and dried.

### EXAMPLE 3

The procedure of Example 2 is employed with the following resin solutions:

|   |        |                                                                          |
|---|--------|--------------------------------------------------------------------------|
| A | 75 g/l | of a 1:1 mixture of dimethylolethylene urea and dimethylolpropylene urea |
|   | 20 g/l | $MgCl_2 \cdot 6H_2O$                                                     |
|   | x g/l  | copolymer 34/66                                                          |
| B | 75 g/l | dimethylol methylcarbamate                                               |
|   | 20 g/l | $ZnCl_2$                                                                 |
|   | x g/l  | copolymer 34/66                                                          |
| C | 75 g/l | dimethylol dihydroxyethylene urea                                        |
|   | 15 g/l | $Zn(NO_3)_2 \cdot 6H_2O$                                                 |
|   | x g/l  | copolymer 34/66                                                          |

The results are listed in Tables 2 to 4.

Table 1

|                          | Finished without copolymer addition | Fluorimeter values |       |       |       |  |
|--------------------------|-------------------------------------|--------------------|-------|-------|-------|--|
|                          |                                     | 82/18              | 67/33 | 34/66 | 18/82 |  |
| Washed once              | 24                                  | 82/18              | 67/33 | 34/66 | 18/82 |  |
|                          |                                     | 41                 | 44    | 60    | 58    |  |
| Washed five times at 98° | 29                                  | 44                 | 47    | 58    | 58    |  |

Table 2

| Resin Solution | Number of washes  | Fluorimeter values of Finished Fabric |         |        |        |
|----------------|-------------------|---------------------------------------|---------|--------|--------|
|                |                   | x = 0 g/l                             | 7.5 g/l | 15 g/l | 30 g/l |
| A              | once at 60°       | 26                                    | 55      | 64     | 74     |
|                | five times at 98° | 29                                    | 58      | 63     | 72     |
| B              | once at 60°       | 33                                    | 65      | 69     | —      |
|                | five times at 98° | 42                                    | 67      | 81     | —      |
| C              | once at 60°       | 20                                    | 40      | 56     | 66     |
|                | five times at 98° | 20                                    | 38      | 58     | 70     |

Table 3

| Resin solution | Number of washes  | Dry crease recovery angle of finished fabric (Averages of determinations in the warp and wet directions) |         |        |        |
|----------------|-------------------|----------------------------------------------------------------------------------------------------------|---------|--------|--------|
|                |                   | x = 0 g/l                                                                                                | 7.5 g/l | 15 g/l | 30 g/l |
| A              | Unwashed          | 137                                                                                                      | 137     | 135    | 125    |
|                | once at 60°       | 145                                                                                                      | 147     | 137    | 131    |
|                | five times at 98° | 140                                                                                                      | 139     | 137    | 132    |
| B              | Unwashed          | 141                                                                                                      | 127     | 113    | —      |
|                | once at 60°       | 140                                                                                                      | 130     | 121    | —      |
|                | five times at 98° | 140                                                                                                      | 132     | 119    | —      |
| C              | Unwashed          | 149                                                                                                      | 143     | 140    | 132    |
|                | once at 60°       | 150                                                                                                      | 147     | 142    | 125    |
|                | five times at 98° | 146                                                                                                      | 140     | 140    | 123    |

Table 4

|                |                   | Wet crease recovery angle of finished fabric<br>(Averages of determinations in the warp and weft directions) |         |        |        |
|----------------|-------------------|--------------------------------------------------------------------------------------------------------------|---------|--------|--------|
| Resin solution | Number of washes  | Amount of copolymer 34/66                                                                                    |         |        |        |
|                |                   | X = 0 g/l                                                                                                    | 7.5 g/l | 15 g/l | 30 g/l |
| A              | Unwashed          | 131                                                                                                          | 134     | 136    | 137    |
|                | once at 60°       | 134                                                                                                          | 134     | 137    | 137    |
|                | five times at 98° | 135                                                                                                          | 134     | 137    | 137    |
| B              | Unwashed          | 134                                                                                                          | 133     | 133    | —      |
|                | once at 60°       | 134                                                                                                          | 134     | 134    | —      |
|                | five times at 98° | 133                                                                                                          | 135     | 129    | —      |
| C              | Unwashed          | 133                                                                                                          | 133     | 136    | 136    |
|                | once at 60°       | 138                                                                                                          | 140     | 143    | 139    |
|                | five times at 98° | 136                                                                                                          | 133     | 134    | 138    |

Table 5

|                |                   | Mean crease recovery angle of finished fabric<br>(Averages of the dry and wet crease recovery angles) |         |        |        |
|----------------|-------------------|-------------------------------------------------------------------------------------------------------|---------|--------|--------|
| Resin solution | Number of washes  | Amount of copolymer 34/66                                                                             |         |        |        |
|                |                   | X = 0 g/l                                                                                             | 7.5 g/l | 15 g/l | 30 g/l |
| A              | Unwashed          | 134                                                                                                   | 135     | 135    | 131    |
|                | once at 60°       | 140                                                                                                   | 141     | 137    | 134    |
|                | five times at 98° | 138                                                                                                   | 136     | 137    | 135    |
| B              | Unwashed          | 138                                                                                                   | 130     | 123    | —      |
|                | once at 60°       | 137                                                                                                   | 132     | 128    | —      |
|                | five times at 98° | 136                                                                                                   | 133     | 124    | —      |
| C              | Unwashed          | 141                                                                                                   | 138     | 138    | 134    |
|                | once at 60°       | 144                                                                                                   | 143     | 143    | 132    |
|                | five times at 98° | 141                                                                                                   | 137     | 137    | 130    |

The loss in tensile strength caused by resin finishing is significantly reduced by the inclusion in the finish of an additive according to this invention.

Very similar results to those given above are obtained with cotton fabrics.

Having thus disclosed the invention what we claim is:

1. In a process for the resin finishing of cellulosic fabrics and cellulosic blend fabrics by padding the fabric with an aqueous solution of (a) an N-methylol or a lower N-alkoxymethyl compound and (b) an acid curing catalyst for the N-methylol or N-alkoxymethyl compound and treating the fabric at 120 to 180°C. to cure the resin, the improvement whereby the affinity of the fabric for anionic optical brighteners is increased which comprises including in said solution (c) a copolymer consisting of N-vinylpyrrolidone units and at least 5.5 weight percent vinyl alcohol units, said components (a), (b), and (c) being present in the solution in amounts of 50-150 g/l, 5-30 g/l, and 3-50 g/l, respectively.

2. A process according to claim 1 wherein the copolymer contains 5.5 to 55 weight percent of vinyl alcohol units.

3. A process according to claim 1 wherein the padded fabric is dried before the resin is cured.

4. A process according to claim 1 wherein the copolymer has a molecular weight in the range 5,000 to 50,000.

5. A process according to claim 1 wherein the copolymer consists of 5.5 to 55 weight percent vinyl alcohol units and 94.5 to 45 weight N-vinylpyrrolidone

units and has a molecular weight in the range 5,000 to 50,000.

6. A process according to claim 1 wherein the copolymer (c) is the reaction product of N-vinylpyrrolidone and vinyl acetate.

7. A composition comprising an aqueous solution of (a) an N-methylol or a lower N-alkoxymethyl compound, (b) an acid curing catalyst for the N-methylol or N-alkoxymethyl compound, and (c) a copolymer consisting of N-vinylpyrrolidone units and at least 5.5 weight percent vinyl alcohol units, said components (a), (b), and (c) being present in amounts of 50-150 g/l, 5-30 g/l, and 3-50 g/l, respectively.

8. A composition according to claim 7 wherein the copolymer has a molecular weight in the range 5,000 to 50,000.

9. A composition according to claim 7 wherein the copolymer (c) is the reaction product of N-vinylpyrrolidone and vinyl acetate.

10. Fabric of cellulosic fibre or cellulose-containing blended fibres having crease resistance and improved affinity for anionic optical brighteners and produced by the process of claim 1.

11. A composition consisting essentially of an aqueous solution of (a) an N-methylol or a lower N-alkoxymethyl compound, (b) an acid curing catalyst for the N-methylol or N-alkoxymethyl compound, and (c) a copolymer consisting of N-vinylpyrrolidone units and at least 5.5 weight percent vinyl alcohol units, said components (a), (b) and (c) being present in amounts of 50-150 g/l, 5-30 g/l, and 3-50 g/l, respectively.

\* \* \* \* \*